

## UNITED STATES PATENT OFFICE

WILLIAM H. FURNESS, OF NATIONAL PARK, NEW JERSEY, ASSIGNOR, BY MESNE ASSIGNMENTS, TO FURNESS CORPORATION, OF PHILADELPHIA, PENNSYLVANIA, A CORPORATION OF NEW JERSEY

## ART OF SILK MANUFACTURE

No Drawing.

Application filed December 12, 1927. Serial No. 239,615.

This invention relates to improvements in the art of silk manufacture and particularly in the manufacture of cuproammonium silk.

In the manufacture of such silk a copper-hydrate-ammonia-cellulose solution is introduced through a suitable spinneret into an alkaline precipitating bath, such, for example, as a caustic bath.

The bath is usually about a 24% caustic 10 solution. A solution of this strength is employed in order to keep the copper soluble and thus prevent it from being precipitated on the thread, the guides and other parts.

The deposition of copper which occurs 15 when employing weak solutions results in a number of disadvantages, among which the following may be mentioned: the thread cannot be wound upon the spool or bobbin without sticking thereto and without sticking of 20 the strands of thread, the thread is opaque, and the finished or conditioned thread is fuzzy.

If the solution could be weak, a great saving 25 in expense would result, due to the relatively small amount of caustic soda carried by the thread and to the saving in the amount of acid required to remove the caustic soda and the copper hydrate; and it is the primary purpose of the present invention to effect this 30 saving and to permit of the employment of a relatively weak caustic solution without encountering the difficulties hereinabove noted.

Other advantages of the invention will appear 35 hereinafter.

In carrying out my invention I reduce the percentage of caustic soda in the solution and employ an additional substance or substances which are unaffected by the caustic 40 soda and which will have the effect of keeping the copper soluble. As one such substance or material, I propose glycerine and in the preferred form of my invention I employ a solution containing about 1% glycerine, 10% caustic and the balance water.

As the filaments are spun into this solution and the thread is formed, some of the copper and ammonia enter the bath and apparently the glycerine unites with the copper hydroxide, caustic soda and ammonia in a soluble 50 form. In any event, I find that the copper does not deposit on the thread and guides, and the thread is clear and does not adhere to the spool or bobbin nor do the strands of the thread being laid upon the spool adhere to one another. Consequently, the above 55 mentioned solution is especially useful in the manufacture of fine filament silk, that is to say, a product having filaments of about two and one-half denier or less and also of fine 60 counts (denier of the thread). Heretofore, great difficulty has been encountered in the production of such fine filament rayon, primarily because of breakage of the fine filaments in the spinning. The product has been 65 objectionably fuzzy, due to the presence of broken filaments. Apparently the glycerine strengthens the precipitating action and im- 70 parts firmness and strength to the filaments, making it possible to spin and twist the filaments into the thread without breakage of the filaments. Because of this the thread, after it has been decotted, washed and dried, is free 75 from fuzz. Furthermore, the glycerine seems to reduce the amount of oxidation which occurs in the thread in the presence of air and caustic soda and a spool can stand for a great many hours without any deterioration.

In addition to the foregoing advantages, I find that the costs are still further reduced by virtue of the fact that I am enabled to obtain substantially complete recovery. Thus, when the bath becomes objectionably laden with copper and ammonia, I remove the ammonia by applying a heat, after which 80 I precipitate copper, as, for example, by adding formaldehyde, which precipitates the copper in the form of copper-oxide. This leaves the caustic and glycerine in solution 85 ready for reuse by proper concentration. 90

While I have specifically mentioned glycerine for the purposes of my invention, it is to be understood that I am not limited to the employment thereof.

5 What I claim is:—

The method of preventing precipitation of copper during precipitation of suproammomium silk thread, which includes spinning the thread in a precipitating bath containing about 1% of glycerin and about 10% of caustic soda.

In testimony whereof I have hereunto signed my name.

15

WILLIAM H. FURNESS.

20

25

30

35

40

45

50

55

60

65